

## UNITED STATES PATENT OFFICE

2,069,790

## LUBRICANT

Eric Wahlforss, Cleveland, Carl L. Johnson,  
Bedford, and George Lacy, Cleveland, Ohio, as-  
signors to The Glidden Company, Cleveland,  
Ohio, a corporation of Ohio

No Drawing. Application October 10, 1934,  
Serial No. 747,766

12 Claims. (Cl. 87—9)

This invention relates to lubricants of the type designed for use in the extreme pressure field, and has particular reference to a new composition which gives exceptional film strength, adhesion and resistance to abrasion. In particular, it contemplates the use of a chlororetene as an addition agent to lubricating oil, to produce a lubricant satisfactory for extreme pressure work, and for machine cutting, threading, etc.

For most common purposes, the ordinary petroleum base lubricating oils are satisfactory. With very rapidly moving machinery, and especially with gears of the hypoid and herring-bone type, extremely high pressure is developed; and the ordinary oil lubricants lack sufficient film strength to maintain a continuous film on this type of gearing. For example, a straight Pennsylvania lubricating oil of 155 seconds Saybolt at 210° F. will only resist pressures up to 8,000 to 9,000 pounds per square inch, while these gears develop pressures requiring lubricants able to resist up to 20,000 pounds and higher. With the acceptance of these gears by automotive engineers for common use on automobile rear ends, a demand has arisen for cheap, effective, extreme pressure lubricants of high film strength. Various products have been suggested and used, with partial satisfaction only.

Halogenation of the lubricating oil itself has been suggested. This is unsafe, as the aliphatic halides formed tend to hydrolyze under adverse conditions, making the lubricant acid and corrosive to the gear surfaces.

Ortho-dichlor benzene has been suggested, but its low boiling point (352° F.) and its low viscosity at elevated temperatures (34-36" Saybolt at 210° F.) are objectionable, its tendency to evaporate being the most important factor against its use.

The chlor-naphthalenes have been used, but optimum results cannot be obtained owing to the limited solubility in most lubricating oils.

In our co-pending application Serial Number 716,004, of which this application is a continuation in part, we disclosed that monochlororetene (in combination with lubricating oils) makes very good extreme pressure lubricants, combining high film strength, excellent adhesion, good viscosity at elevated temperatures, good miscibility with lubricating oil, low vapor tension, and resistance to hydrolysis, with reasonable cost and availability.

Monochlororetene is at ordinary temperatures a pale amber, viscous liquid which possesses perfect miscibility with lubricating oil. It boils at

about 215° C. at 4 mm. pressure and has a viscosity of 54-58 seconds Saybolt at 210° F. It is extremely stable, as it may be boiled for hours with caustic solution without any indication of hydrolysis. Its adhesion to metal is outstandingly good.

On mixing small percentages of monochlororetene with lubricating oil, a noticeable increase in film strength is obtained. This increases in almost a straight line relationship until a blend of approximately 15% monochlororetene and 85% lubricating oil is obtained (about 2% total chlorine) the curve then flattens out almost to a horizontal line.

We have now found that when the polychlorinated retenes are used, together with lubricating oils, in the preparation of extreme pressure lubricants, even better results are obtained, as to film strength and other desirable properties, than with the monochlororetene lubricants. As the degree of substitution increases, the maximum film strength obtainable increases, the film strength obtainable with hexachlororetene being more than double that obtainable with the monochloro compound.

While monochlororetene has been prepared in the past, and may be rather easily prepared and purified, the polychlororetenes are new compounds which are somewhat more difficult to purify. The dichlor compound may be prepared by direct chlorination of melted retene, and purified by washing or by vacuum distillation; but the tri and higher chloro compounds decompose on vacuum distillation and cannot be easily prepared from the molten retene, due to foaming of the reaction mix. The preferred method of making these compounds is to chlorinate in the presence of a solvent, preferably an equal volume of carbon tetrachloride. The crude product, containing asphaltic material, hydrochloric acid, chlorinated retene and solvent, is then purified, separating the solvent, acid and asphaltic material from the polychlor compound. One method is to steam distill off solvent and acid, and dissolve the residue in petroleum naphtha; the insoluble asphalts are then separated from the solution, and the solvent is removed from the polychlororetene by distillation. Further washing with water and/or dilute caustic soda solution, to remove any possible traces of acid, may be resorted to, but is in general not essential to obtaining a pure product on the lower chlor compounds. This washing is very helpful, however, on the more highly chlorinated compounds.

Another method is to filter the reaction mixture

through fuller's earth. Asphaltic material is filtered off, and free acid is absorbed; the solution of chlororetene may then be treated to remove the solvent, to give a fairly pure technical product.

5 The dichloro compound is a very viscous oil; and the products range through plastic solids to the hexa chloro compound, which is a hard resinous material, with a ball and ring melting point of 138-142° F. It powders readily, but the powder 10 tends to sinter somewhat at high summer heats (ca. 90° F.) All of the compounds are completely soluble in lubricating oil.

10 The following examples will indicate the superior results obtained with our new lubricating 15 compositions:

*Example 1*

454 grams of monochlororetene were mixed with 2,500 grams of Pennsylvania #150 (viscosity 150 20 seconds Saybolt @ 210° F.) bright stock, to give a mixture containing 2% chlorine. The resultant lubricant was tested on a Timken Lubricant Tester (the standard device for testing lubricants of the extreme pressure type), giving an O. K. load of 33 pounds (approximating a pressure of 20,000 25 pounds per square inch) and a score load of 38 pounds (22,500 pounds per square inch). A reduction to 1½% chlorine content in the mixture 30 reduced the lubrication under load considerably; increase to 3% chlorine content resulted in no increase in load values.

A six hour run at 33 pounds load gave an abrasion of .0045 gram; after the 6 hour test, the original results were obtained on the O. K. and 35 score loads, demonstrating the stability of the compound under load conditions over a period of time.

*Example 2*

171 grams of dichlororetene, prepared by chlorination in solvent, and subsequent purification by 40 steam distillation, naphtha solution, filtration and solvent evaporation, were mixed with 2,500 grams of Pennsylvania #150 bright stock (the standard lubricating oil used on the Timken Tester) and 45 the lubricant obtained, containing 1½% chlorine was tested as in Example 1. An O. K. load of 25 pounds (15,000 pounds per square inch pressure) and a score load of 33 pounds (20,000 pounds per 50 square inch pressure) was obtained. A blend of the 234 grams of dichlororetene with 2,500 grams of the same oil (chlorine content 2%) gave a 38 pound O. K. load (22,500 pounds per square inch pressure) and a score load of 43 pounds (25,000 pounds per square inch pressure).

55 *Example 3*

118 grams of hexachlororetene, purified as was 60 the dichloro compound of Example 2, with the further step of washing with dilute caustic and water, was blended with 2,500 grams of the Pennsylvania #150 bright stock, to give a 2% chlorine content. An O. K. load of over 100 pounds (approximating 57,000 pounds per square inch pressure) was obtained, with no scoring. The machine was run 6 65 hours with a 33 pound load; an abrasion loss of .0035 gram was found. After the test, the compound was again subjected to the 100 pound load, and found O. K.

70 *Example 4*

A blend similar to that of Example 3 was made up, using a hexachlororetene purified as in Example 3, but with the final caustic wash omitted. An O. K. load of 77 pounds (45,000 pounds per 75 square inch pressure) was obtained, with a score

load of 86 pounds (50,000 pounds per square inch pressure). A 6 hour run at 33 pound load gave .0045 gram abrasion; a test after the abrasion run gave the same O. K. and score loads as originally.

5 Other chlorinated retenes give results which vary from those obtained with the mono compound, to those which are obtained with the highest chlor compound we have tested—hexachlororetene; and our results indicate that as the chlorination of the retene molecule is increased, the possible film strength obtainable is increased, without increasing the amount of chlorine in the finished lubricant. The amount of addition agent needed is, of course, reduced as the chlorination 10 is increased. A 2% chlorine content in the lubricant requires, on a 2,500 gram basis, only 118 grams of the hexachloro compound, against 454 grams of the mono compound.

15 A further advantage in using the polychloro 20 compounds lies in their superior non-volatility. While the monochloro compound is relatively non-volatile, boiling at 642° F. under normal pressure, with decomposition, the polychloro compounds become less and less volatile, the hexa compound being to all intents entirely non-volatile. This reduces loss of film strength during prolonged use.

25 Unlike some other series of chlorinated compounds, the chlororetene retain their good oil-solubility even in the higher chloro compounds. 30 This is, of course, a prime essential in compounds which are to be mixed with lubricating oil.

35 As indicated by the abrasion test, a properly purified polychlororetene lubricant is as resistant to hydrolysis as the monochlororetene lubricant.

40 While we have shown in our examples only the tests with Pennsylvania #150 bright stock, the polychlororetene may be employed with other lubricating oils, and with blended compositions and greases, compounded from Mid-Continent, 40 California, or foreign crudes.

45 Although particularly intended for extreme pressure work, our lubricating compositions may, of course, be used for other purposes, as for auto cylinder oil, cutting oil, etc. In these cases, 45 thinner oils should be used than for extreme pressure work. The adhesion of our lubricants, and their resistance to high pressures, make them especially valuable in the preparation of cutting oils; while small quantities of the polychloro 50 retene, added to ordinary cylinder stock, improve the lubricating properties considerably.

55 Polychlororetene, as defined in the claims, means an individual compound, or a mixture of the polychlororetene.

We claim:

1. A lubricant comprising a hydrocarbon lubricant material and a chloro derivative of retene.
2. A lubricant comprising a hydrocarbon oil and a chlororetene.
3. A lubricant comprising a mixture of hydrocarbon oil and chlorinated retene, the chlorine content of the mixture being about 2%.
4. A lubricant comprising a hydrocarbon lubricant material and a polychlororetene.
5. A lubricant comprising a hydrocarbon oil and a polychlororetene.
6. A lubricant comprising a hydrocarbon oil and a polychlororetene, the chlorine content of the mixture being about 2%.
7. A lubricant comprising a hydrocarbon lubricant material and dichlororetene.
8. A lubricant comprising a hydrocarbon lubricant material and hexachlororetene.
9. A lubricant comprising a hydrocarbon lu-

- bricant material and dichlororetene, the chlorine content of the mixture being about 2%.
10. A lubricant comprising a hydrocarbon lubricant material and hexachlororetene, the chlorine content of the mixture being about 2%.
- 5 11. A lubricant comprising a hydrocarbon lubricant material and monochlororetene.

12. A lubricant comprising a hydrocarbon lubricant material and monochlororetene, the chlorine content of the mixture being about 2%.

ERIC WAHLFORSS. 5  
GEORGE LACY.  
CARL L. JOHNSON.